

No. 650,710.

Patented May 29, 1900.

H. DUNLOP.

ROADWAY.

(Application filed June 27, 1899.)

(No Model.)



Witnesses:

George A. Brereton.

Wall O. Brereton.

Inventor:

Hugh Dunlop,

by E. F. Munglock Co.  
his Attorneys.

# UNITED STATES PATENT OFFICE.

HUGH DUNLOP, OF SYDNEY, NEW SOUTH WALES.

## ROADWAY.

SPECIFICATION forming part of Letters Patent No. 650,710, dated May 29, 1900.

Application filed June 27, 1899. Serial No. 722,094. (No model.)

*To all whom it may concern:*

Be it known that I, HUGH DUNLOP, residing at 43 Sloane street, Summer Hill, Sydney, in the Colony of New South Wales, have invented 5 a certain new and useful Roadway, of which the following is a description.

My invention relates to roadways having wooden paving-blocks as a foundation, my object being to provide an efficient and durable covering for the blocks, which produces a good roadway and also preserves the wood.

To these ends my invention consists in the various matters hereinafter described and claimed.

15 The drawing illustrates in sectional elevation a portion of a roadway constructed in accordance with the present invention.

In carrying out my invention I employ two mixtures or divisions, which I shall hereinafter 20 call the "first" and "second" mixtures.

To make the first mixture, I employ the following ingredients in the proportions indicated, viz: two hundredweight of blue-metal screenings, one hundredweight Portland cement, one-half ( $\frac{1}{2}$  cwt.) hundredweight caustic soda, three hundredweight resin, and two hundredweight calcined clay. To mix these together, the resin and caustic soda are boiled 25 in water, and when cooled the mixture is combined with the Portland cement, calcined clay, and blue-metal screenings.

To make the second mixture, I employ the following ingredients in the proportions indicated, viz: two hundredweight of bitumen, 35 (placed in a boiler or vat,) one hundredweight of resin, two and one-half ( $2\frac{1}{2}$ ) gallons boiled linseed-oil, and twelve gallons of Stockholm tar. When these ingredients are boiled to a thoroughly-liquid state, I add two hundred- 40 weight calcined clay, two hundredweight of blue-metal screenings, and any quantity of sand that may be deemed necessary.

I first coat the blocks with the first mixture and allow the same to remain about six hours 45 to solidify in order to form a preservative for the blocks and also to act as a gripper to the

second mixture. After the first mixture has solidified I apply the second mixture by pouring it over the first mixture (already set) in a hot liquid state, (by any approved means,) 50 and after this second mixture has been laid on and sufficient time allowed for it to cool it is rolled until it becomes an even surface. It is then covered with sand and again rolled, this sanding and rolling being repeated as 55 often as may be required, and in from four to six days this improved composition for covering wood blocks will be solid, and the roadway thus formed will allow of the heaviest traffic passing over it without in any way destroying or damaging it. 60

The thickness of the compositions when set on wood blocks is about half an inch, according to the requirements of the place, so that besides being very efficacious it will be found 65 also to be a very economical top dressing.

Having now particularly described and ascertained the nature of my said invention and in what manner the same is to be performed, I desire to state I do not in any way claim the 70 use of wood blocks in the formation of roadways and foot-paths; but

What I claim is—

In a roadway or the like, a layer of wooden paving-blocks, a composition adjacent to and covering said blocks, said composition being composed of the following ingredients, viz., blue-metal screenings, Portland cement, caustic soda, resin and calcined clay, and a second composition adjacent to and covering 75 80 said first-mentioned composition, said second composition being composed of the following ingredients, viz., bitumen, boiled linseed-oil, resin, Stockholm tar, calcined clay, blue-metal screenings and sand; substantially as 85 described.

In testimony whereof I have hereunto set my hand this 7th day of March, 1899.

HUGH DUNLOP.

Witnesses:

JAMES BAKER,  
ROBERT MALLENSON.